

## UNITED STATES PATENT OFFICE

2,445,826

## ELECTROLYTE PURIFICATION IN MANGANESE ELECTROWINNING

William L. Hammerquist, Knoxville, Tenn., assignor to Electro Manganese Corporation, Knoxville, Tenn., a corporation of Delaware

No Drawing. Application February 1, 1944,  
Serial No. 520,689

10 Claims. (Cl. 204—105)

1

This invention relates to purification of solutions for use as electrolytes in the electrodeposition including the electrowinning of manganese.

In the electrowinning of manganese, electrolytic cells are employed in which the electrolyte is divided into catholyte and anolyte. A type of cell in commercial use at the present time contains a plurality of catholyte chambers suspended in a tank containing anolyte liquid. A cathode in sheet form is suspended in each catholyte chamber and these chambers include in their structure permeable diaphragms which separate the catholyte liquid from the anolyte liquid. The anodes are suspended in the anolyte liquid in spaced relation to the adjacent diaphragm walls so that the cell comprises a series of anodes and cathodes alternately arranged in a row and separated by the catholyte or diaphragm chambers.

Anolyte containing manganese sulfate, ammonium sulfate, and sulfuric acid is withdrawn from the anolyte chamber and used to extract manganese ore and the extract is then subjected to purification. When purified it becomes catholyte liquid and is supplied to the catholyte chamber. Metallic manganese is deposited on the cathodes in the cathode chambers. The cathodes are commonly made in sheet form from a suitable metal or alloy. At the end of a predetermined plating period, the cathodes with a deposit of manganese metal thereon are removed from the cathode chambers, the electrolytic deposit is stripped therefrom, and the cathodes after suitable reconditioning are returned to the cell.

In the catholyte chamber the catholyte is partially depleted of its contents of manganese. It then passes to the anolyte chamber partly or wholly by diffusion and/or partly by other means of transfer, as, for example, overflow, and becomes anolyte liquid. There is thus a circulation of liquid from the anolyte chamber to the catholyte chamber and back to the anolyte chamber, and in the course of this circulation outside the cell, the anolyte liquid is enriched in manganese by contact with suitably prepared manganese ore, or by the addition of the manganese sulfate from a source other than manganese ore, and subjected to purification.

It will thus be seen that to the circulating stream outside the cell, there is continuously added a source of manganese, and since such sources contain substances other than manganese which may be generally referred to as impurities, it will be clear that these impurities are being continuously added to the circulating stream. Such impurities may include iron, arsenic, anti-

2

mony, cobalt, nickel, copper, molybdenum, and zinc, and it has been found necessary either to remove these impurities completely or else reduce them to such small or insignificant proportions that they do not interfere with the plating process and the production of suitably pure electrolytic manganese. The latter in its commercial form must be extremely pure, e. g., of the order of 99.95% manganese, and in this form has a characteristic bright, metallic luster.

It has been discovered that soluble or colloidal silica is an impurity, the removal or control of which is highly desirable because of its adverse effects on obtaining satisfactory cathodic deposition. Having arrived at this knowledge, the invention then proceeds further and applies a remedy, this remedy being the use of a reagent which is effective in separating silica from the solution intended for use as catholyte, at least to an extent sufficient to prevent the above-mentioned phenomenon. The reagent which has so far been found best adapted for the purpose is aluminum sulfate. This occurs in various forms, as, for example, the anhydrous salt, or the salt containing water of crystallization, or in the form of various double salts. In accordance with the invention, an aluminum sulfate reagent is applied to the solution to be purified at a pH range of about 5.5 to 7.5.

30 In the commercial electrowinning process where ore is used as the source of manganese, the latter is extracted with anolyte at a pH which may be from 1 to 3, after which the pH is raised to about 5.5 to 6.5, and air or other suitable oxidizing agent is employed to oxidize the iron to the ferric condition and cause the precipitation thereof, together with any arsenic, antimony, and the like which may be present. The iron precipitate and gangue may be separately removed, and are preferably removed together, and the resulting solution or mother liquid having a pH of about 5.5 to 6.5 may, as pointed out in co-pending abandoned application of Karl M. Leute, Serial No. 461,110, filed October 7, 1942, 35 be treated for the removal of cobalt and nickel, for which purpose the pH is raised to about 7.2 to 7.5 and treated with a precipitant, e. g., ammonium sulfide, for cobalt, nickel, and other heavy metals whose sulfides are insoluble at this pH range. Since it has been found desirable to effect the aluminum sulfate treatment at a pH of about 5.5 to about 7.5, this treatment may conveniently be carried out on the mother liquor after separation of the iron precipitate and gangue and having a pH of about 5.5 to 6.5.

Thereafter the pH may be raised to about 7.2 to 7.5 for precipitation of the cobalt and nickel. A portion of the aluminum sulfate may be added at the lower pH range of about 5.5 to 6.5, and the remainder at a higher range of about 6.5 to 7.5. Still another variation is to add all or a part of the aluminum sulfate to the mother liquor after separation of the iron precipitate and gangue at a pH range of about 5.5 to 6.5, and the remainder may be added after the pH has been increased to about 7.2 to 7.5 preparatory to precipitating the cobalt, nickel, etc.

It is also possible to add the aluminum sulfate at any time prior to iron precipitation and filtration, as, for instance, during the ore leaching operation. This method, however, is deemed wasteful since aluminum begins to precipitate as hydrous oxide at a pH of 3, and the aluminum thus precipitated in the presence of large amounts of precipitated iron and gangue cannot perform its function efficiently. To attain maximum efficiency from the aluminum in removing silicates, it should be precipitated from the solution in the absence of such foreign materials as precipitated iron and gangue and at a pH not lower than about 5.5 or higher than about 7.5. Practical considerations do not always permit such ideal conditions, and operations may have to be carried out under less favorable conditions.

The addition of the aluminum sulfate causes the formation of the precipitate of aluminum hydroxide which has been found effective in eliminating soluble or colloidal silica to a sufficient extent.

Proportions of aluminum sulfate varying from about 10 to 20 parts by weight of anhydrous aluminum sulfate for every one hundred thousand parts by weight of solution, have been found adequate. In general, about twenty to twenty-five pounds of 57 per cent. aluminum sulfate to about ten thousand gallons of solution weighing about ten pounds per gallon, have been found sufficient.

However, as shown in column 3 of the table at the end of the specification and in the paragraph following that table, proportions of aluminum sulfate (calculated as anhydrous aluminum sulfate) as high as  $40.0 \times 20 = 800$  pounds of aluminum sulfate per 10,000 gallons of solution may be used and since a gallon of said solution weighs 10 pounds, the proportion of said aluminum sulfate may be as high as 800 pounds per 100,000 pounds of said solution.

The precipitate formed by the addition of the aluminum sulfate may be separated as such prior to the separation of cobalt, nickel, etc. Preferably, however, the precipitate of aluminum hydroxide is formed prior to or concurrently with the sulfide precipitate and the two removed at the same time and by the same means, as, for example, by filtration. In some cases treatment of the solution with aluminum sulfate may occur after separation of the cobalt, nickel, etc.

There are, of course, numerous specific variants of the manner of adding the aluminum sulfate, and all such variants are intended to be included, provided the precipitation occurs within a pH range of about 5.5 to 7.5.

It is to be understood that the invention is not limited to the purification of solutions obtained by extracting manganese-containing ore with sulfuric acid solutions or with anolyte, and is generally applicable to the treatment of solutions containing manganese sulfate in order to purify

said solutions and adapt them for use as catholyte.

It is, of course, entirely possible to replenish the manganese content of the anolyte by enriching it with manganese sulfate obtained from any suitable source, and the invention includes, in general, the treatment of solutions containing manganese sulfate in order to purify them to obtain catholyte liquid. Whether or not the solution is obtained by extracting ore, it may well contain silica in soluble or colloidal form, that is to say, silica in a highly dispersed condition, which exists either in the form of a true solution or a colloidal solution, and the invention in its generic aspects is directed to treatment of solutions to separate the silica of that type therefrom. While impurities other than silica are commonly present in solutions for the electrodeposition including the electrowinning of manganese, the invention is not in its generic aspects limited to the removal of silica in conjunction with the elimination of the other impurities, e. g., iron, cobalt, and nickel, but, rather, to the removal of silica whether or not it may be associated with other impurities. Therefore, any specific description of embodiments of the invention which includes the treatment of manganese-containing ore and the removal of impurities other than silica, are not to be regarded as limitations in respect of the generic phase of the invention. It is also to be pointed out that in some cases manganese may be electroplated in a cell not provided with a diaphragm, that is to say, in contradistinction to the process of electrowinning of manganese from solutions containing manganese salts and/or from manganese-containing ores, it is quite possible to carry out a manganese electroplating process in which manganese is deposited as a coating on various objects. Here, also, it is necessary to employ a pure electrolyte, and the invention is applicable to the purification of solutions for the electrodeposition of manganese whether that deposition be an electroplating process or an electrowinning process. Therefore, it will be understood that while the specific description of the invention is in terms of an electrowinning process, that specific description is not to be regarded as a limitation on the generic features of the invention.

A typical example of an embodiment of the invention may be described as follows:

Anolyte liquid having a composition of about 10 to 18 grams per liter of manganese as manganese sulfate, about 120 to 180 grams per liter of ammonium sulfate and a pH of about 1 to 2, is withdrawn from the anolyte chamber of a commercial cell employed for the electrowinning of manganese and is mixed with manganese ore in a digester, the ore being suitably conditioned, if necessary (e. g., by the process described in the co-pending application of Elmer M. Wanamaker et al., Serial No. 497,352, filed August 4, 1943, now Patent 2,397,824, granted April 2, 1946), and, as a result of agitation with the ore, a mixture of ore and extract is obtained, the extract having a concentration of manganese of about 20 to 50 grams per liter. The pH of the extract is adjusted to about 5.5 to 6.5, and air or other suitable oxidizing agent is employed to oxidize iron to the ferric condition and cause precipitation thereof along with any arsenic, antimony, or the like which may be present. The insoluble gangue and iron precipitate is then separated, as by filtration, and a solution is obtained. To this solution, which weighs about ten pounds per

gallon, there is added aluminum sulfate in the proportion of about twelve and one-half pounds, calculated as 57 per cent. aluminum sulfate, for each ten thousand gallons of solution, which is equivalent to a concentration of anhydrous aluminum sulfate of about seven and one-eighth pounds per one hundred thousand pounds of solution. This addition may occur at a pH of about 5.5 to about 7.5, a typical pH value being about 6.3 and a typical range being about 6.0 to 6.5. A precipitate is formed which is preferably allowed temporarily to remain in suspension. Thereafter the pH of the liquid is raised to about 7.2 to about 7.5 and an additional twelve and one-half pounds of 57 per cent. aluminum sulfate is added. Thus the total amount of aluminum sulfate added in the two steps is equivalent to fourteen and one-quarter pounds of anhydrous aluminum sulfate for each ten thousand gallons of solution. Subsequently a precipitant for cobalt, nickel, etc., e. g., ammonium sulfide, is added, precipitating the cobalt, nickel, etc., in the form of their insoluble sulfides mixed with the aluminum hydroxide precipitate caused by the addition of the aluminum sulfate. The mixed precipitate is then removed, as by filtration or other suitable means, and the purified liquid is then in suitable condition for use as catholyte.

In the preferred embodiment of the invention, sufficient precipitant is used to reduce the content of soluble or colloidal silica to not more than about 0.001 gram per liter before using the purified solution as catholyte. For this purpose the solution to be purified may be analyzed to determine its content of said soluble or colloidal silica and an amount of aluminum sulfate added not less than 4.0 parts by weight of aluminum sulfate (100%) for each part by weight of colloidal and/or soluble silica, or about 7.0 parts by weight of commercial aluminum sulfate containing 57%  $\text{Al}_2(\text{SO}_4)_3$ .

The following table shows the minimum concentrations of aluminum sulfate, calculated as anhydrous or 100%  $\text{Al}_2(\text{SO}_4)_3$  and expressed as grams per liter (and pounds per 10,000 gallons of solution), necessary to precipitate varying concentrations of soluble or colloidal silica expressed as grams per liter:

| g./l. of Soluble or Colloidal Silica | g./l. of $\text{Al}_2(\text{SO}_4)_3$ , calc. as Anhydrous | lbs. $\text{Al}_2(\text{SO}_4)_3$ per 10,000 gallons of solution calc. as Anhydrous |
|--------------------------------------|------------------------------------------------------------|-------------------------------------------------------------------------------------|
| 0.001                                | 0.0040                                                     | 0.40                                                                                |
| 0.002                                | 0.0080                                                     | 0.80                                                                                |
| 0.003                                | 0.0120                                                     | 1.20                                                                                |
| 0.004                                | 0.0160                                                     | 1.60                                                                                |
| 0.005                                | 0.0200                                                     | 2.00                                                                                |
| 0.006                                | 0.0240                                                     | 2.40                                                                                |
| 0.007                                | 0.0280                                                     | 2.80                                                                                |
| 0.008                                | 0.0320                                                     | 3.20                                                                                |
| 0.009                                | 0.0360                                                     | 3.60                                                                                |
| 0.010                                | 0.0400                                                     | 4.00                                                                                |
| 0.020                                | 0.0800                                                     | 8.00                                                                                |
| 0.030                                | 0.1200                                                     | 12.00                                                                               |
| 0.040                                | 0.1600                                                     | 16.00                                                                               |
| 0.050                                | 0.2000                                                     | 20.00                                                                               |
| 0.060                                | 0.2400                                                     | 24.00                                                                               |
| 0.070                                | 0.2800                                                     | 28.00                                                                               |
| 0.080                                | 0.3200                                                     | 32.00                                                                               |
| 0.090                                | 0.3600                                                     | 36.00                                                                               |
| 0.1000                               | 0.4000                                                     | 40.00                                                                               |

Larger excesses over the minimum proportions of aluminum sulfate above set forth are desirable, e. g., excesses of, say, 2 to 20 fold.

What is claimed is:

1. The process of treating a solution to be used as an electrolyte in the electrodeposition includ-

ing the electrowinning of manganese, said solution containing manganese sulfate, ammonium sulfate and soluble silica, which comprises treating said solution at a pH of about 5.5 to 7.5 with aluminum sulfate in the proportion of not less than four parts by weight of aluminum sulfate calculated as anhydrous aluminum sulfate for each part by weight of soluble silica, forming a precipitate, and separating said precipitate from said solution.

2. In the process of manganese electrowinning involving the use of an electrolytic cell in which the electrolyte is divided into catholyte and anolyte and in which process anolyte liquid is withdrawn from the cell and used to extract manganese-containing ore to produce an extract which is subjected to purification for use as catholyte, said purification including precipitation of the iron, separation of the iron precipitate and gangue, and the production of a solution from which said iron precipitate and gangue have been separated, said solution containing soluble silica, the improvement which comprises treating said solution with aluminum sulfate in the ratio of not less than four parts by weight of aluminum sulfate calculated as anhydrous aluminum sulfate for each part by weight of soluble silica at a pH of about 5.5 to 7.5, forming a precipitate, and separating said precipitate.

3. In the process of manganese electrowinning involving the use of an electrolytic cell in which the electrolyte is divided into catholyte and anolyte and in which process anolyte liquid is withdrawn from the cell and used to extract manganese-containing ore to produce an extract which is subjected to purification for use as catholyte, said purification including precipitation of the iron, separation of the iron precipitate and gangue, and the production of a solution from which said iron precipitate and gangue have been separated, said solution containing soluble silica, the improvement which comprises treating said solution with aluminum sulfate in the ratio of about 10 to 20 parts by weight of aluminum sulfate calculated as hydrous aluminum sulfate to about one hundred thousand parts of said solution at a pH of about 5.5 to 7.5 and thereafter treating said solution with a precipitant for cobalt and nickel within said pH range, forming a precipitate, and separating said precipitate from said solution.

4. In the process of manganese electrowinning involving the use of an electrolytic cell in which the electrolyte is divided into catholyte and anolyte and in which process anolyte liquid is withdrawn from the cell and used to extract manganese-containing ore to produce an extract which is subjected to purification for use as catholyte, said purification including precipitation of the iron, separation of the iron precipitate and gangue, and the production of a solution from which said iron precipitate and gangue have been separated, said solution containing soluble silica, the improvement which comprises treating said solution with aluminum sulfate in the ratio of about 10 to 20 parts by weight of aluminum sulfate calculated as anhydrous aluminum sulfate to about one hundred thousand parts of said solution, adding said aluminum sulfate at a pH of about 5.5 to 6.5, then raising the pH to about 7.2 to 7.5, forming a precipitate, and separating said precipitate from said solution.

5. In the process of manganese electrowinning involving the use of an electrolytic cell in which the electrolyte is divided into catholyte and an-

lyte and in which process anolyte liquid is withdrawn from the cell and used to extract manganese-containing ore to produce an extract which is subjected to purification for use as catholyte, said purification including precipitation of the iron, separation of the iron precipitate and gangue, and the production of a solution from which said iron precipitate and gangue have been separated, said solution containing soluble silica, the improvement which comprises treating said solution with aluminum sulfate in the ratio of about 10 to 20 parts by weight of aluminum sulfate calculated as anhydrous aluminum sulfate to about one hundred thousand parts of said solution, adding a portion of said aluminum sulfate at a pH of about 5.5 to 6.5, then raising the pH to about 7.2 to 7.5 and adding the remainder of the aluminum sulfate, forming a precipitate, and separating the precipitate from the solution.

6. The process of treating a solution to be used as an electrolyte in the electrodeposition including the electrowinning of manganese, said solution containing manganese sulfate, ammonium sulfate and soluble silica, which comprises treating said solution at a pH of about 5.5 to 7.5 with aluminum sulfate in the proportion of not less than four parts by weight of aluminum sulfate calculated as anhydrous aluminum sulfate for each part by weight of soluble silica, forming a precipitate, treating said solution with a precipitant for cobalt and nickel within said pH range to precipitate cobalt and nickel, and separating the combined precipitates.

7. Process of treating a solution to be used as an electrolyte in the electrodeposition including the electrowinning of manganese, said solution containing manganese sulfate, ammonium sulfate, and soluble silica, which comprises treating said solution at a pH of about 5.5 to 7.5 with aluminum sulfate in the proportion of not less than about 4 milligrams of aluminum sulfate per liter of said solution (0.40 pound per 10,000 gallons of said solution) for each milligram per liter (0.00001 pound per gallon) of said silica, the said aluminum sulfate being calculated as anhydrous aluminum sulfate.

8. Process of treating a solution to be used as an electrolyte in the electrodeposition including the electrowinning of manganese, said solution containing manganese sulfate, ammonium sulfate, soluble silica and the sulfates of cobalt and nickel, which comprises treating said solution at a pH of about 5.5 to 7.5 with aluminum sulfate in the proportion of not less than about 4 milligrams of aluminum sulfate per liter of said solution for each milligram per liter of said silica, the said aluminum sulfate being calculated as anhydrous aluminum sulfate, to form a precipitate of aluminum hydroxide, adding ammonium

sulfide to precipitate to sulfides of cobalt and nickel mixed with the aluminum hydroxide precipitate, and separating the said mixture of precipitates.

5. The process of treating a solution to be used as an electrolyte in the electrodeposition including the electrowinning of manganese, said solution containing manganese sulfate, ammonium sulfate and soluble silica, which comprises treating said solution at a pH of about 5.5 to 7.5 with aluminum sulfate in the proportion of about 10 to 800 parts by weight of aluminum sulfate calculated as anhydrous aluminum sulfate to about 100,000 parts by weight of said solution, thereby 10 forming a silica precipitate, and separating said precipitate from said solution.
10. In the process of manganese electrowinning involving the use of an electrolytic cell in which the electrolyte is divided into catholyte and anolyte and in which process anolyte liquid is withdrawn from the cell and used to extract manganese-containing ore to produce an extract which is subjected to purification for use as catholyte said purification including precipitation of the iron, separation of the iron precipitate and gangue, and the production of a solution from which said iron precipitate and gangue have been separated, said solution containing soluble silica, the improvement which comprises 20 treating said solution with aluminum sulfate in the ratio of about 10 to 800 parts by weight of aluminum sulfate calculated as anhydrous aluminum sulfate to about 100,000 parts by weight of said solution at a pH of about 5.5 to 7.5 and thereafter treating said solution with a precipitant for cobalt and nickel within said pH range, forming a precipitate, and separating said precipitate from said solution.
- 25

40 WILLIAM L. HAMMERQUIST.

#### REFERENCES CITED

The following references are of record in the file of this patent:

#### UNITED STATES PATENTS

| Number       | Name             | Date          |
|--------------|------------------|---------------|
| 1,137,005    | Jacobson         | Apr. 27, 1915 |
| 1,843,006    | Stevens et al.   | Jan. 26, 1932 |
| 50 1,989,603 | Nicoll           | Jan. 29, 1935 |
| 2,266,137    | Westby           | Dec. 16, 1941 |
| 2,267,831    | Liebknecht       | Dec. 30, 1941 |
| 2,325,723    | Wanamaker et al. | Aug. 3, 1943  |
| 2,340,188    | Jukkola          | Jan. 25, 1944 |

#### OTHER REFERENCES

Industrial and Engineering Chemistry, vol. 31, July 1939, pp. 859, 860, 861.

Water Works Engineering, Oct. 13, 1937, pp. 1514, 1517.